

## 1

3,536,527

MEANS AND METHOD FOR REDUCING SPARKING IN CATHODE RAY TUBES  
Laszlo Javorik and Otto Laudi, Chicago, and Robert A. Mitchell, Berwyn, Ill., assignors to National Video Corporation, Chicago, Ill., a corporation of Illinois  
No Drawing. Filed Sept. 11, 1967, Ser. No. 667,331  
Int. Cl. B44d 1/02

U.S. Cl. 117—216

2 Claims

### ABSTRACT OF THE DISCLOSURE

An anti-sparking coating for the interior of a cathode ray tube which is applied over the usual electrically conductive carbonaceous coating, the supplemental coating consisting essentially of aluminum hydroxide and a soluble silicate.

### SUMMARY OF THE INVENTION

Cathode ray tubes conventionally have an interior coating of an electrically conductive carbonaceous material. Commonly used for this purpose is a product known as "Aquadag" and commonly referred to throughout the television industry as "dag." The carbonaceous layer extends from near the edge of the funnel portion of the tube back into the gun portion and serves as a means for conducting electric current to apply a potential of the order of 25 kv. to the electron gun. Frequently during the life of such a tube, particles of the "dag" become detached from the coating and result in interior sparking or arcing and consequently, a poor television picture. We have found that through the use of a supplemental coating, particularly one compatible with the usual "dag" coating, this problem can be resolved. We find that a coating made up of aluminum hydroxide and a soluble silicate is particularly advantageous for this purpose. A specific example of the practice of the invention is set forth below.

### EXAMPLE

For the purpose of preparing the anti-sparking coating material, we use one part by weight of deionized water with one part by weight of purified gelatinous aluminum hydroxide. This mixture is placed within a ball mill using porcelain balls and milled for 24 hours at room temperature (68–78° F.). Thereafter the suspension so achieved was mixed by taking 25 parts by volume of the aluminum hydroxide suspension and mixed with 75 parts by volume of potassium silicate solution (electronic grade),

## 2

the potassium silicate solution having a specific gravity of 1.26. This mixture was agitated for one hour and thereafter sprayed thoroughly and evenly over the inner dag surface (which was previously baked to its final condition) using airless spray apparatus. The supplemental coating was then baked dry in conventional fashion.

With the foregoing coating, we find that if there is any tendency of the multiple-coating to flake, it occurs in the aluminum oxide which will not cause sparking.

While in the foregoing specification a detailed description of an embodiment of the invention has been set down for the purpose of illustration, many variations in the details herein given may be made by those skilled in the art without departing from the spirit and scope of the invention.

We claim:

1. In a cathode ray tube having an enlarged portion at one end providing a front viewing screen and a reduced portion at the other end housing an electron gun, said tube having an interior electrically conductive carbonaceous coating extending rearwardly from said screen, the improved supplemental coating interiorly of and on said carbonaceous coating and consisting essentially of about 25 parts by volume of aluminum hydroxide and about 75 parts by volume of potassium silicate.

2. In a method for suppressing sparking in cathode ray tubes having an electrically conductive carbonaceous layer on the tube interior extending rearwardly from the front viewing screen, the steps of spraying over said layer an aqueous mixture consisting essentially of about 25 parts by volume of aluminum hydroxide and about 75 parts by volume of potassium silicate, the said potassium silicate having a specific gravity of about 1.26, and thereafter drying the sprayed mixture.

### References Cited

#### UNITED STATES PATENTS

|           |         |                 |       |           |
|-----------|---------|-----------------|-------|-----------|
| 2,223,924 | 12/1940 | Stephan         | ----- | 313—64 X  |
| 2,496,901 | 2/1950  | Van Hoorn       |       |           |
| 2,951,773 | 9/1960  | Helle et al.    | ----- | 117—226 X |
| 3,108,906 | 10/1963 | Scharrer et al. | ----- | 117—226   |

ALFRED L. LEAVITT, Primary Examiner

C. K. WEIFFENBACH, Assistant Examiner

U.S. Cl. X.R.

29—25.11; 117—96, 97, 104, 219, 223, 224; 313—64